

June 27, 1944.

E. J. JACOB

2,352,201

COMPOSITION OF MATTER

Filed May 23, 1941



Fig. 1.



Fig. 2.



Fig. 3.



Fig. 4.

BY

INVENTOR:  
Ezekiel J. Jacob  
Michael S. Drinan  
his agent

## UNITED STATES PATENT OFFICE

2,352,201

## COMPOSITION OF MATTER

Ezekiel J. Jacob, New York, N. Y., assignor to  
Benjamin Liebowitz, New York, N. Y.

Application May 23, 1941, Serial No. 394,893

5 Claims. (Cl. 131—230)

My present invention relates to a new composition of matter, and more particularly to a material of which bowl-shaped receptacles for smoking pipes may be made.

An object of my present invention consists in providing a new heat resistant composition of matter which, at the same time, is strong and porous.

A further object of my invention consists in providing a slowly setting cold binding cement or like material.

Another object of my invention consists of a new material for pipe bowls or the like which, after a few smokes, acquires a brownish, meerschaum-like color.

Still another object of my present invention consists in providing for pipe bowls or the like a new material which is heat insulating and thereby protects the surrounding material. This object is of particular significance at the time of this application when the importation of the hard briar woods usually employed in smokers' pipes is substantially cut off and when more extensive use of domestic woods may be necessitated.

With the above objects in view, my present invention mainly consists of a new composition of matter, particularly for bowl-shaped receptacles for smoking pipes, comprising a heat resistant cementing substance mixed with fine heat resistant filaments. A preferred embodiment of my invention consists of a composition of matter comprising mainly plaster of Paris, intimately mixed with fine glass filaments.

The expression "heat resistant" as used throughout this specification, means having the ability to withstand at least a temperature which is equal to the temperature encountered in the bowl of a smoking pipe, due to the burning tobacco therein, without undergoing any substantial physical or chemical change.

Another word frequently used in this specification and claims, whose meaning should be clarified, is "cementing substance." This expression, as used throughout this specification, embraces any bonding material capable of retaining heat resistant fine filaments, for instance glass filaments, within its structure. Such cementing substances are, for example, cold binding materials as cement, plaster of Paris, and hot binding material as low firing clay, or the like. Furthermore, it is possible to use as cementing substances materials which may be brought into the desired shape by compression, for instance, plastics incorporating briar dust, wood dust or the

like. In all cases, however, it is important that the cementing substance be heat resistant in the above defined sense.

As stated above, various cementing substances may be used; but for convenience of description, I will describe my invention in combination with plaster of Paris.

As fine heat resistant filaments I prefer to use glass filaments having a diameter of the order of magnitude of a few ten-thousandths of an inch. These filaments are used in discontinuous state. I have found that by intimately mixing the cementing substance, preferably plaster of Paris, with discontinuous fine glass filaments, these filaments hold the plaster particles during hardening apart from each other, thereby increasing its porosity after hardening.

The filaments used by me, particularly the glass filaments, are resilient to a certain extent and thus they also increase the resiliency and strength of the hardened cementing substance. Therefore, the tendency of an article, e. g. a pipe or a pipe bowl made of such a substance, to break during use is substantially decreased.

As stated above, a preferred embodiment of my invention consists of a composition of matter comprising plaster of Paris and discontinuous fine glass filaments. After hardening of the plaster of Paris, the glass filaments should be substantially evenly distributed through it and firmly embedded therein.

I have found that by adding silica gel to the plaster of Paris it is possible to prevent it from being calcined when exposed to damp heat: the silica gel particles embedded in the plaster of Paris, will adsorb the moisture and retain it, thereby avoiding calcination.

This tendency of silica gel makes its addition to materials from which pipe bowls of the like are made, particularly important and advantageous; the condensates formed during smoking are adsorbed by the silica gel contained in the pipe bowl, preventing thereby calcination of the material of which the pipe bowl is made. Furthermore, the tarry liquids and condensates adsorbed by the silica gel are forming a brownish deposit, which gives the inner surface of a pipe bowl made of plaster of Paris with addition of silica gel even after a relatively short period of smoking a meerschaum-like appearance.

I have furthermore found that by addition of a small percentage of Congo-red, the setting of the plaster of Paris can be retarded; thus, by addition of a small percentage, e. g. less than 1 per cent of Congo-red, it is possible to attain

slow setting of the plaster of Paris. Furthermore, another effect of the Congo-red is to produce a material of considerably greater hardness and mechanical strength.

It should be noted that the percentage of the ingredients of the new composition of matter may be varied to a wide extent: thus, the same may comprise from 50-95% of plaster of Paris, from 50-5% of fine heat resistant filaments, preferably glass filaments, from 0.1 to 5% of silica gel, and from 0.1 to 2% of Congo-red.

My invention will be more clearly understood from the accompanying drawing, in which:

Fig. 1 is a perspective view of a cube made of my new composition of matter;

Fig. 2 is a bowl-shaped element adapted to lie within the bowl of a smoking pipe and to receive and to hold the tobacco;

Fig. 3 is a pipe provided with a lining for the pipe bowl; and

Fig. 4 is a cross-section through the bowl-shaped element shown in Fig. 3.

In the embodiment shown in Fig. 1, my new composition of matter consists of discontinuous glass filaments 1 embedded in hardened plaster of Paris 2; the glass filaments 1 are thoroughly mixed with the plaster of Paris, in either dry or wet state; I prefer to mix the glass filaments with a thick paste of semi-hardened plaster of Paris, as I have found that in this case cohesion of the dry glass filaments by static electricity can easily be avoided.

Figs. 2 and 4 show a bowl-shaped element fitting into a pipe bowl and holding the tobacco while it is smoked. At the bottom of this bowl-shaped element an opening 3 may be provided, if required. In the side wall of the bowl, an opening 4 is arranged; this opening 4 has to be in register with pipe stem 5, indicated in Fig. 2 by dotted lines.

Instead of making a bowl-shaped element which has to be inserted into the wooden pipe bowl, I may also make the pipe bowl entirely of new material proposed by me.

The pipe shown in Fig. 3 consists of a stem 6 and a pipe bowl 7. The inner surface of this bowl is covered by a lining 8 consisting of my

new composition of matter. In order to obtain a uniform lining, I propose first to pour the lining material while still in liquid state into the pipe bowl, let it set in the pipe bowl for some time, and pour the material which has not set, again out of the bowl. The material set on the inner surface of the wooden bowl 7, then forms a lining 8 of uniform thickness.

The specific embodiments shown are merely illustrative.

What I claim as my invention and desire to secure by Letters Patent of the United States is:

1. Composition of matter, particularly for bowls of smoking pipes, comprising plaster of Paris intimately mixed with fine heat resistant filaments and Congo-red.

2. Composition of matter, particularly for bowl-shaped receptacles of smoking pipes adapted to hold the tobacco while it is smoked, said composition of matter comprising hardened plaster of Paris, discontinuous fine glass filaments, and a small percentage of Congo-red, said glass filaments and said Congo-red substantially evenly distributed through said hardened plaster of Paris.

3. Composition of matter, particularly for bowls of smoking pipes, comprising plaster of Paris, intimately mixed with fine heat resistant filaments, silica gel, and Congo-red.

4. Composition of matter, particularly for bowl-shaped receptacles of smoking pipes adapted to hold the tobacco while it is smoked, said composition of matter comprising hardened plaster of Paris, discontinuous fine glass filaments, silica gel, and a small percentage of Congo-red, said glass filaments, silica gel, and Congo-red substantially evenly distributed through said hardened plaster of Paris.

5. Composition of matter, particularly for bowl-shaped receptacles of smoking pipes adapted to hold the tobacco while it is smoked, said composition of matter comprising from fifty to ninety-five per cent of plaster of Paris, from fifty to five per cent of fine glass filaments, from 0.1 to five per cent of silica gel, and from 0.1 to 2 per cent of Congo-red.

EZEKIEL J. JACOB.